

May 2, 1961

E. PELZEL

2,982,677

BEARING ALLOYS

Filed Oct. 10, 1957



Inventor  
Erich Pelzel

By  
Wenderoth, Lind & Ponack  
Atty's.

## 1

2,982,677

## BEARING ALLOYS

Erich Pelzel, Stolberg, Rhineland, Germany, assignor to Vereinigte Oesterreichische Eisen- und Stahlwerke Aktiengesellschaft, Linz-Donau, Austria, an Austrian company

Filed Oct. 10, 1957, Ser. No. 689,374

13 Claims. (Cl. 148—13)

Many binary alloys in the solid state consist of mixed crystals, i.e., atomic solutions which exist only within a definite temperature range.

Similar relationships occur in the zinc/aluminium system with an aluminium content above 17% Al. In the accompanying drawing, a section of the zinc/aluminium phase diagram is illustrated. Alloys over 17% Al solidify to  $\beta$  mixed crystals, line  $a-b$ . If the proportion of aluminium is between 17 and 21%, the zinc crystals precipitate on further cooling, whereas the aluminium content of the  $\beta$  mixed crystals increases to 21% Al, line  $a-c$ . This step is completed at 275° C. At this temperature, the  $\beta$  mixed crystals decompose to a eutectoid "C." Alloys with more than 21% Al decompose on further cooling, line  $c-d$ , to two kinds of mixed crystals, that having the higher Zn content likewise decomposing to the eutectoid "C" at 275° C. Aluminium/zinc alloys with an aluminium content between 17 and 21% hence consist of zinc crystals and eutectoid, of 21% of only eutectoid and above 21% of eutectoid and aluminium-rich  $\beta$  mixed crystals.

With pure aluminium/zinc alloys, the eutectoid decomposition occurs rapidly, but is hindered by additions of Mg, Cu and similar elements.

Quenched alloys show increased strength properties, quenching after longer heating above 275° C. thus representing an improvement step.

Alloys which largely or wholly consist of  $\beta$  mixed crystals have proved suitable as bearing alloys. In particular, with alloys with more than 30% Al, a Cu content of  $\frac{1}{6}$  to  $\frac{1}{4}$  of the Al content and the remainder zinc, a reduction in strength and hardness by destructive heating between 80° and 280° C. causes a surprising improvement in bearing properties, if it is assumed that these include a lower coefficient of friction and increased emergency running properties. Also in oil-less running, shafts and journals are not worn away, whereas this is the case with improved alloys and those which were rapidly cooled by casting.

Furthermore, a bearing alloy with an Al/Cu/Zn basis was proposed, which contained 3–15% Al, 0.001–2% Cu, 0.01–0.06% Mn and as the remainder zinc with less than 0.01 each of Sn, Pb and Cd. This alloy shows no marked emergency running properties.

It was also known that alloys with 80–85% Zn, 14–19% Al and 1–2% Cu or with 80–85% Zn, 14–18% Al and 0–6% Cu exhibit unusual tensile strength and hardness and are especially suitable for manufacturing die cast articles, drawn rods and sheets.

It has now been found that alloys with 16–29% Al and certain copper contents, remainder zinc, give good bearing materials if the destructive heating is carried out suitably. This was surprising to the technician, since it was previously believed with high aluminium contents that there was a proportion of  $\beta$  mixed crystals, which in the alloy range according to the invention is slight or even nil. In this range, the eutectoid structure is mainly

## 2

prevalent. All attempts to use alloys according to the invention as bearing materials fail on the lesser emergency running property, since the importance of the destructive heating is not recognised. It is shown namely that with 5 copper-containing alloys with more than 16% Al the natural cooling in sand or permanent molds is insufficient to lead to decomposition into a fine-grained eutectoid, and the cooled alloy must be subjected to a subsequent heating from room temperature.

10 An example shows the effect. An alloy of 21% Al, 5% Cu and 74% Zn (99.99% pure) was cast into billets in a sand mould. The strength test gave a breakage strength of 40 kg./mm.<sup>2</sup>, an elongation of 5% and a Brinell hardness of 130 kg./mm.<sup>2</sup>. Bushes were made 15 from the billets and were run in a corresponding arrangement under a constant bearing pressure and velocity with oil lubrication. After closing off the oil supply, the temperature of the bearing rose from 60° C. to 320° C. in 80 seconds, the bearing journals were worn and the machine stopped. The same alloy was subjected to a 12-hour heating at 200° C. The mechanical properties had 20 worsened. The breakage strength was 30 kg./mm.<sup>2</sup>, the elongation 5% and the Brinell hardness only 100 kg./mm.<sup>2</sup>. Bushings were made from the billets and subjected 25 to the same running test. On closing off the oil supply, the temperature rose from 50° C. to 220° C., but only after 300 seconds, the friction resistance strongly increased and a grey, greasy paste formed on the bearing surface, so that no wearing of the journal occurred.

30 The example shows that the heating causes a lessening of the mechanical properties, but also a definite improvement of the bearing properties.

The method of manufacturing bearing alloys with good 35 emergency running properties by heating zinc/aluminium/copper alloys at temperatures between 150° and 275° C. gives the best results with alloys of 16–29% Al, a copper content which is between  $\frac{1}{10}$  and  $\frac{1}{4}$  of the aluminium content and is at least 2.2% and the remainder zinc (99.99% pure). In particular, the alloys between 40 20 and 22% Al, a copper content of  $\frac{1}{10}$  to  $\frac{1}{4}$  of the aluminium content and the remainder zinc give a considerable 45 emergency running capacity, wherein the alloy mentioned in the example with 21% Al, 5% Cu, 74% pure zinc shows in sand moulding and chill moulding and also in the pressed state the optimum emergency running capacity after destructive heating.

According to the invention, a method is provided for manufacturing a bearing material based on a Zn/Al/Cu alloy, in which an alloy containing 16–29% Al,  $\frac{1}{10}$  to 50  $\frac{1}{4}$  of the aluminium content of Cu, but at least 2.2% Cu, and the remainder zinc is subjected after casting or pressing to a heat treatment at temperatures from 150° to 275° C. for 2 to 90 hours duration.

The alloys must be manufactured with fine zinc with 55 a purity grade of at least 99.9% Zn, wherein the remainder may consist of 0.080% lead, less than 0.005% tin and less than 0.020% cadmium. In the main, as the cadmium and tin contents are lower, the lead content can be higher (Pb max. 0.1 with Cd=0, Sn=0). The 60 alloys may further contain no magnesium content over 0.01%, preferably not over 0.005%, and no iron content above 0.1%.

The temperature range for economically acceptable 65 heating times 170°–275° C., but with lower temperatures longer heating times can be used. The heating time is not only dependent upon the heating temperature but also upon the copper content. The values given in the following table for the heating temperature represent merely 70 optimum values and the invention is not limited to them. The table principally illustrates the connection between the heating temperature, the copper content and the

heating time. As the example given above indicates, shorter heating times suffice to give usable results.

| Heating temperature, ° C. | Heating time in hours |                        |
|---------------------------|-----------------------|------------------------|
|                           | Cu = $\frac{1}{4}$ Al | Cu = $\frac{1}{10}$ Al |
| 270                       | 6                     | 3                      |
| 250                       | 12                    | 6                      |
| 200                       | 24                    | 15                     |
| 170                       | 36                    | 22                     |
| 150                       | 60                    | 32                     |

The clearly more satisfactory results with a copper content of  $\frac{1}{10}$  the aluminium content correspond to lower hardness of the alloy.

If the recommended heating is carried out more than once, a further important advantage for the bearing properties of the metal alloys is a successive lowering of the thermal coefficient of expansion with the number of heatings. Whereas a non-tempered material in the region of from 20-100° C. has a linear thermal coefficient of expansion of  $23-25 \times 10^{-6}$ , the latter diminishes with further heating to  $20-22 \times 10^{-6}$ . After a second heating, it diminishes to  $18-20 \times 10^{-6}$ . The effect of further heatings is always less and it depends upon the particular intended purpose of how far the diminution so obtained is in a definite relation to the greater consumption, e.g. for precision bearings. As to the hardness of the alloys, a copper content of  $\frac{1}{4}$  to  $\frac{1}{6}$  of the aluminium content is best.

In order to accelerate the decomposition process on heating, the temperature can fluctuate during the heating between 150° and 275° C. With this fluctuating heating, the temperature naturally must not go below 150° C. nor rise above 275° C., but the temperature can fluctuate over a range which lies between these two values.

A case hardening, i.e. heating above 275° C., by which the structure becomes homogenised, is to be avoided, since an alloy of the desired composition with a homogeneous structure is unsuitable as a bearing material.

Finally, it may be mentioned that it has not previously been possible to determine exactly whether the eutectoid shown in the diagram at c is obtained with 21% or 22% Al. The value of 21% is therefore to be considered only as an approximation.

I claim:

1. A method of manufacturing a bearing material without homogenisation of the alloy structure thereof, which comprises subjecting a Zn/Al/Cu alloy, containing from 16 to 29% aluminum, at least 2.2% copper, the copper content being from  $\frac{1}{10}$  to  $\frac{1}{4}$  of the aluminum content, and the remainder zinc, to pressing, and heat treating the resulting alloy at a temperature from 150° to 275° C. for a period of from 2 to 90 hours, whereby case hardening is avoided.

2. A method of manufacturing a bearing material without homogenisation of the alloy structure thereof, which comprises forming a Zn/Al/Cu alloy containing from 16 to 29% aluminum, at least 2.2% copper, the copper content being from  $\frac{1}{10}$  to  $\frac{1}{4}$  of the aluminum content, and the remainder zinc, and heat treating the formed resulting alloy at a temperature from 150° to 275° C. for a period of from 2 to 90 hours.

3. A bearing made of a Zn/Al/Cu alloy having a non-homogenised alloy structure and containing from 16 to 29% aluminum, at least 2.2% copper, the copper content being from  $\frac{1}{10}$  to  $\frac{1}{4}$  of the aluminum content, and the remainder zinc, said alloy having been heat treated at a temperature of from 150° to 275° C. for a period of from 2 to 90 hours.

4. A bearing cast from a Zn/Cu/Al alloy having a non-homogenised alloy structure and containing from 16 to 29% aluminum, at least 2.2% copper, the copper content being from  $\frac{1}{10}$  to  $\frac{1}{4}$  of the aluminum content, and the remainder zinc, to casting, and heat treating the resulting alloy at a temperature from 150° to 275° C. for a period of from 2 to 90 hours.

tent being from  $\frac{1}{10}$  to  $\frac{1}{4}$  of the aluminum content, and the remainder zinc, the cast alloy having been subjected to a temperature of from 150° to 275° C. for a period of from 2 to 90 hours.

5. A method of manufacturing a bearing material without homogenisation of the alloy structure thereof, which comprises subjecting a Zn/Al/Cu alloy, containing from 16 to 29% aluminum, at least 2.2% copper, the copper content being from  $\frac{1}{10}$  to  $\frac{1}{4}$  of the aluminum content, and the remainder zinc, to casting, and heat treating the resulting alloy at a temperature from 150° to 275° C. for a period of from 2 to 90 hours, whereby case hardening is avoided.

15. 6. A method according to claim 5 wherein the alloy contains from 18 to 26% aluminum.

7. A method according to claim 5 wherein the copper content of the alloy amounts to  $\frac{1}{4}$  to  $\frac{1}{6}$  of the aluminum content.

20. 8. A method of manufacturing a bearing material without homogenisation of the alloy structure thereof, which comprises subjecting a Zn/Al/Cu alloy, containing from 20 to 22% aluminum, at least 2.2% copper, the copper content being from  $\frac{1}{10}$  to  $\frac{1}{4}$  of the aluminum content, and the remainder zinc, to casting, and heat treating the resulting alloy at a temperature from 200° to 270° C. for a period of from 3 to 24 hours.

25. 9. A method according to claim 8 wherein the copper content of the alloy amounts to  $\frac{1}{4}$  to  $\frac{1}{6}$  of the aluminum content.

30. 10. A method of manufacturing a bearing material without homogenisation of the alloy structure thereof, which comprises subjecting a Zn/Al/Cu alloy, containing from 16 to 29% aluminum, at least 2.2% copper, the copper content being from  $\frac{1}{10}$  to  $\frac{1}{4}$  of the aluminum content, and the remainder zinc, to casting, and heat treating the resulting alloy at least twice at a temperature from 150° to 275° C. for a period of from 2 to 90 hours each.

35. 11. A method of manufacturing a bearing material without homogenisation of the alloy structure thereof, which comprises subjecting a Zn/Al/Cu alloy, containing from 16 to 29% aluminum, at least 2.2% copper, the copper content being from  $\frac{1}{10}$  to  $\frac{1}{4}$  of the aluminum content, and the remainder zinc, to casting, and heat treating the resulting alloy at a temperature fluctuating within the range of from 150° to 275° C. for a period of from 2 to 90 hours.

40. 12. A method of manufacturing a bearing material without homogenisation of the alloy structure thereof, which comprises subjecting a Zn/Al/Cu alloy, containing from 20 to 22% aluminum, a copper content from  $\frac{1}{4}$  to  $\frac{1}{6}$  of the aluminum content and the remainder zinc, to casting, and separately heat treating the resulting alloy at least twice at a temperature within the range of from 200° to 270° C. for a period of from 3 to 24 hours each.

45. 13. A method of manufacturing a bearing material without homogenisation of the alloy structure thereof, which comprises subjecting a Zn/Al/Cu alloy, containing from 20 to 22% aluminum, a copper content from  $\frac{1}{4}$  to  $\frac{1}{6}$  of the aluminum content and the remainder zinc, to casting, and heat treating the resulting alloy at a temperature fluctuating within the range of from 200° to 270° C. for a period of from 3 to 24 hours.

#### References Cited in the file of this patent

##### FOREIGN PATENTS

748,871 Great Britain May 16, 1956  
70 528,372 Canada July 31, 1956

##### OTHER REFERENCES

Principles of Physical Metallurgy, 3rd ed., pp. 198 and 200, G. E. Doan, 1953.